

# United States Patent [19]

Kobayashi et al.

[11] 3,763,003

[45] Oct. 2, 1973

[54] METHOD FOR PRODUCING FERRITE THIN FILM BODY

[75] Inventors: Seihin Kobayashi; Michihiro Torii; Katsuyuki Oshima, all of Hamana-gun Shizuoka-ken, Japan

[73] Assignee: Fuji Denki Kagaku Kabushiki Kaisha, Tokyo, Japan

[22] Filed: June 8, 1971

[21] Appl. No.: 151,069

## [30] Foreign Application Priority Data

June 11, 1970 Japan 45/50454

[52] U.S. Cl. 204/37 R, 117/62, 148/121, 204/192

[51] Int. Cl. C23b 5/52

[58] Field of Search 117/62, 71 M; 148/121, 204/37 R, 192; 75/125

## [56] References Cited

### UNITED STATES PATENTS

2,443,756 6/1948 Williams 204/37 R  
3,148,079 9/1964 Banks et al. 117/62

3,625,849 12/1971 Rogalla 204/37 R  
3,549,428 12/1970 Lommel 148/121

## FOREIGN PATENTS OR APPLICATIONS

153,342 12/1961 U.S.S.R. 204/37 R

## OTHER PUBLICATIONS

Koretzky, H. "Electrodeposition of Permanent Magnetic Materials." IBM Technical Disclosure Bulletin, Vol. 6, No. 8, 1/64. 204/37R.

Primary Examiner—John H. Mack

Assistant Examiner—W. I. Solomon

Attorney—Eliot S. Gerber

## [57] ABSTRACT

A method for producing a ferrite thin film body is provided which comprises the steps of separately applying each of the metals composing the ferrite in layers on a non-magnetic heat-resistant substrate, subjecting the metallic layers to a diffusion reaction under inert gas at an elevated temperature to produce a diffused solid solution, and subjecting the diffused solid solution to oxidation at an elevated temperature for a time period sufficient to change the solid solution to a ferrite body.

9 Claims, 1 Drawing Figure

PATENTED OCT 2 1973

3,763,003



## METHOD FOR PRODUCING FERRITE THIN FILM BODY

This invention relates to a method for producing a ferrite thin film body, to be used mainly as memory elements, and more particularly to a method wherein each of the metals composing the ferrite is separately applied, in layers, on a non-magnetic heat-resistant substrate and then are subjected separately to diffusion and oxidizing reactions.

Conventionally, vacuum evaporation and a spattering method have been used to produce ferrite thin film body on a non-magnetic heat-resistant substrate, the substrate having, for example, the form of a wire or a plate. In the vacuum evaporation method, the metals composing the ferrite are heated enough to be evaporated and are solidified, under vacuum, on the substrate to form alloy layers thereon. The alloy layers are subjected to an oxidizing reaction to form the ferrite thin film body on the substrate.

In the spattering method, positive ions generated by a cold cathode discharge in an inert gas are collided against a ferrite body and, thereby, the spattered metals composing the ferrite are deposited on the substrate to form a ferrite thin film body thereon.

But, many disadvantages have been experienced in the ferrite thin film bodies produced in accordance with the above-mentioned methods. Firstly, as each of the metals composing the ferrite exists on the substrate in its amorphous state, the density of the crystallized particles is low, sintering reaction is delayed, the demagnetizing field becomes strong, and the ratio of input/output shows a very undesirable value. Secondly, in the oxidizing process, the metals composing the ferrite may separate from the substrate. Thirdly, the surface of the produced ferrite thin film body is not even. Fourthly, it is very difficult to reproduce the ferrite thin film body of same composition.

Furthermore, it seems that the undesirable properties of the conventional ferrite thin film bodies are caused by fine cracks formed on the surface of the ferrite thin film body while the metals composing the ferrite on the substrate is concurrently subjected to diffusion and oxidation reactions.

Accordingly, these conventional methods are undesirable and are not acceptable to produce the ferrite thin film body of high reliability.

An objective of the present invention is to provide a method for producing a ferrite thin film body of high reliability and free from the above-mentioned disadvantages.

According to the present invention, the method for producing ferrite thin film body comprises the step of separately applying each of the metals composing the ferrite in layers on a non-magnetized heat-resistant substrate, subjecting the metallic layers to a diffusion reaction under inert gas at an elevated temperature to form a diffused solid solution, and subjecting the diffused solid solution to oxidation at an elevated temperature for a time period sufficient to change the solid solution to a ferrite body.

In order to separately apply each of the metals composing the ferrite in layers on the substrate, conventional methods of electric plating, vacuum evaporation, cold cathode discharge spattering or the like can be successfully employed. Preferably, the substrate is made of a platinum wire or an alumina-ceramic wire.

In the diffusion process, the metallic layers composing the ferrite on the substrate are exposed to an inert gas at an elevated temperature so as to change the metallic layers to a solid solution. During the diffusion process, an electric current is applied to both of the metallic layers and the substrate.

After the diffusion reaction, the diffused solid solution on the substrate is reacted with oxygen at an elevated temperature, for a period long enough to change the diffused solid solution to ferrite thin film body.

By separately applying each of the ferrite composing metals in layers to the substrate, it becomes easy to control the ratio of composing metals and, thereby, to reproduce ferrite thin film bodies having the same compositions. Furthermore, as the metallic layers are subjected to the diffusion reaction (to make the diffused solid solution before the oxidizing process) many advantages are obtained, such that (a) the ferrite thin film body is even and dense, (b) the ferrite thin film body

20 will not be separated from the substrate, providing a reliable ferrite thin film body, (c) the sintering reaction is speedily effected, and (d) the demagnetizing field is reduced to remarkably improve the ratio of input/output.

25 Taking an example of Cu—Mn ferrite, which is widely known as one of the materials having a rectangular magnetic characteristic, an embodiment of the present invention shall be described hereinafter with reference to the drawing, in which:

30 The single drawing is a graph showing the characteristics of pulse drive currents applied to a Cu—Mn ferrite thin film body, produced in accordance with the present invention.

### EXAMPLE

Platinum wire is used as a substrate. Layers of metal are applied to the wire, by electrochemical plating, in the order of Fe (Iron), Cu (Copper), and Mn (Manganese). The following table shows the conditions and materials of each of the separate electric plating baths:

| Fe                | Cu                 | Mn                |                    |                    |                    |
|-------------------|--------------------|-------------------|--------------------|--------------------|--------------------|
| FeSO <sub>4</sub> | 370g/l             | CuCN              | 20g/l              | MnCl <sub>2</sub>  | 350g/l             |
| FeCl <sub>3</sub> | 30g/l              | NaCN              | 40g/l              | NH <sub>4</sub> Cl | 200g/l             |
| NH <sub>4</sub> C | 23g/l              | NaCO <sub>3</sub> | 15g/l              | KCNS               | 2g/l               |
| PH                | 4.5                | PH                | 11.5               | PH                 | 5.0                |
| Temp.             | 40°C               | Temp.             | 60°C               | Temp.              | 20°C               |
| D.K               | 8A/dm <sup>2</sup> | D.K               | 8A/dm <sup>2</sup> | D.K                | 8A/dm <sup>2</sup> |
| Plating thickness | 0.6μ               | Plating thickness | 0.3μ               | Plating thickness  | 0.6μ               |

55 The plated platinum wire was then placed into a chamber filled with inert gas (containing oxygen less than 2%), such as nitrogen gas or argon gas. The temperature in the chamber was elevated, during 1 hour, up to a temperature higher than 800°C but lower than 1083°C, which is the melting point of Cu. Keeping the chamber at the elevated temperature for an additional 30 minutes, electric current of 1-3 ampere was applied to the platinum wire, as the cathode, and to the plated metallic layers. A diffusion reaction occurred and the metal layers were changed to a solid solution. Then the temperature inside the chamber was lowered to room temperature, the duration of the temperature lowering being 1 hour.

60 After the diffusion reaction step, the inert gas was removed and oxygen substituted (purity of more than 90 percent). The chamber was then heated during one

hour up to 1150°C. The oxidization of the diffused solid solution was effected at the elevated temperature for an additional 15 minutes, during which the solid solution was changed to ferrite thin film body. Thereafter, the produced ferrite thin film body was gradually cooled in air, the cooling occurring for a period of one hour.

As shown in the drawing, the Cu—Mn ferrite film body, produced in accordance with the method of the present invention, has a faster switching time and an excellent rectangular magnetic characteristic and is sufficiently good to be used for magnetic memory elements.

As disclosed above, the method according to the present invention provides reliable ferrite thin film body having excellent magnetic characteristics.

Although the present invention has been described with reference to the preferred embodiment shown in the drawing, many modifications and alternations may be made within the spirit of the present invention.

We claim:

1. A method for producing a Cu-Mn ferrite thin film body on a non-magnetic heat-resistant substrate comprising the steps of applying Fe, Cu, and Mn respectively in layers on said substrate, subjecting said metallic layers to a diffusion reaction under inert gas at a temperature higher than 800°C but lower than 1083°C, said metallic layers being thereby changed to a diffused solid solution, and subjecting said solid solution to oxidation at a temperature higher than 1083°C for a sufficient time to change said solid solution to a ferrite body.

2. A method as claimed in claim 1, wherein said me-

tallic layers and said substrate as the cathode are supplied with electric current while they are subjected to said diffusion reaction.

3. A method as claimed in claim 2, wherein said metallic layers are formed on said substrate, such as wire or plate, by electrochemical plating.

4. A method as claimed in claim 3, wherein said metallic layers are formed on said substrate, such as wire or plate, by vacuum evaporation.

5. A method as claimed in claim 2, wherein said metallic layers are formed on said substrate, such as wire or plate, by a sputtering method.

6. A method for producing a Cu—Mn ferrite thin film body on a non-magnetic heat-resistant substrate comprising the steps of plating Fe, Cu, and Mn respectively in layers on said substrate, subjecting said plated metallic layers to a diffusion reaction under inert gas at a temperature higher than 800°C but lower than 1083°C while said plated metallic layers and said substrate as the cathode are supplied with an electric current, said metallic layers being thereby changed to a diffused solid solution, and subjecting said solid solution to oxidation at a temperature higher than 1083°C for a sufficient time to change said solid solution to a ferrite body.

7. A method as claimed in claim 5, wherein said substrate is a platinum wire.

8. A method as claimed in claim 5, wherein said substrate is an alumina-ceramic wire.

9. A method as claimed in claim 6 wherein the layers are applied in the order of Fe, Cu and Mn.

\* \* \* \* \*

35

40

45

50

55

60

65

UNITED STATES PATENT OFFICE  
CERTIFICATE OF CORRECTION

Patent No. 3,763,003 Dated October 2, 1973

Inventor(s) Seihin Kobayashi; Michihiro Torii; Katsuyuki Oshima

It is certified that error appears in the above-identified patent  
and that said Letters Patent are hereby corrected as shown below:

[30] Foreign Application Priority Data  
changed to  
-- June 10, 1970 Japan ..... 49509 --

Signed and sealed this 19th day of February 1974.

(SEAL)  
Attest:

EDWARD M.FLETCHER, JR.  
Attesting Officer

C. MARSHALL DANN  
Commissioner of Patents